

## UNITED STATES PATENT OFFICE

2,129,422

## COMPOUND FOR LUBRICATING WIRE ROPE

James F. Hall, Columbus, Ohio, assignor to The Ironsides Company, Columbus, Ohio, a corporation of Ohio

No Drawing. Application December 17, 1936,  
Serial No. 116,379

## 2 Claims. (Cl. 87—9)

This invention relates to an improved lubricant adapted for use as a coating material for wire ropes or cables and, more specifically, wire ropes or cables employed in connection with elevators.

- 5 In the manufacture of wire ropes or cables, it is desirable to coat the individual wires and strands thereof with a lubricant which will have the properties of minimizing the actual rubbing together of metallic surfaces, that is, the interengaging surfaces of the individual wires or strands of a composite braided cable, or the contacting of the outer surfaces of such a cable with other associated metallic surfaces, such as guide wheels, pulleys, or drums.
- 10 15 In accordance with the present invention, my improved lubricant is preferably applied to the wire rope or cable during the process of forming the latter but, likewise, is of such composition that it may be used with highly satisfactory results when applied to cables previously manufactured and actually engaged in use.

Inasmuch as wire ropes or cables are usually wound on spools or reels during shipment or storage, it is a further object of the invention to provide an improved lubricant therefor which when applied to the ropes or cables will possess a sufficiently high melting point and other complementary properties of adhesion so that the lubricant will not melt or drip from the cables when subjected to ordinary temperatures.

30 35 Another object of the invention resides in the provision of a lubricant for use in the capacity set forth which when applied to metallic elevator cables imparts sufficient adhesiveness thereto as to minimize any tendency on the part of the rope or cable to slip on the drums or sheaves as the cable is wound or unwound or passes thereabout during elevator operation.

40 45 A still further object of the invention rests in the provision of a lubricant which when applied to a metallic rope or cable of the braided multiple strand type will possess a light amber color when in the form of a thin film on the rope or cable, to the end of permitting easy and convenient inspection of the latter when it is in service.

As illustrative of certain preferred compositions for producing the lubricant comprising the present invention, the following examples are given:

## Example 1

Per cent

|                                             |    |
|---------------------------------------------|----|
| Stearic acid soap                           | 7  |
| Rosin                                       | 4  |
| Rubber cement                               | 2  |
| Petroleum oil (160 sec. Saybolt at 210° F.) | 87 |

The above ingredients may be used with or without the addition of any filler or oxidizing agents.

## Example 2

Per cent 5

|                   |    |
|-------------------|----|
| Stearic acid soap | 7  |
| Rosin             | 4  |
| Petroleum oil     | 89 |

It will be understood that it is within the scope 10 of the present invention to vary somewhat the proportions of the several ingredients set forth.

The general practice for application of this lubricant to a wire rope during its manufacture is to have a small pot or kettle, equipped with a heating means, such as an electric element, steam or direct gas flame, mounted above the forming die for the rope or cable, the kettle allowing the melted lubricant to drip through a regulating valve on the individual wires or strands immediately prior to the passage of the latter into the forming die or dies. I have found that the most effective temperature for heating the lubricant is one of the order of 240° F. The quick setting property of the lubricant results in a thorough 15 and immediate adhesion thereof to the wire 20 strands of the cable.

## What is claimed is:

1. As a new composition of matter, an amber colored lubricant for metallic cables permitting 30 easy inspection of the same comprising a quick setting adhesive mixture including petroleum oil of a viscosity of the order of 160 seconds Saybolt at 210° F. in the proportion of at least 87% together with stearic acid soap, rosin and rubber 35 cement in the respective ratio of 7:4:2, said composition being fluid at a temperature of the order of 240° F.

2. As a new composition of matter, an amber colored lubricant for metallic cables permitting 40 easy inspection of the same comprising a quick setting adhesive mixture including petroleum oil of a viscosity of the order of 160 seconds Saybolt at 210° F. in the proportion of approximately 87% together with approximately 7% stearic acid 45 soap, approximately 4% rosin, and approximately 2% rubber cement, said composition being fluid at a temperature of the order of 240° F.

JAMES F. HALL.

50